

## 1

3,355,389

**DETERGENT BARS HAVING LIME SOAP  
DISPERSING CHARACTERISTICS**

David M. Marquis, Orinda, Calif., assignor to Chevron Research Company, a corporation of Delaware  
No Drawing. Filed July 20, 1964, Ser. No. 383,914  
11 Claims. (Cl. 252—121)

**ABSTRACT OF THE DISCLOSURE**

Detergent bar composition having improved lime soap dispersing property and suitable for use in hard water contained by incorporating a water soluble soap which may contain in addition a water soluble non-soap synthetic detergent in a water soluble salt of thiodisuccinic acid having at least two hydrogen atoms of the carboxyl group replaced by an alkali metal or magnesium as a lime soap dispersant. The amount of the lime soap dispersant being incorporated may be between 5% and 25% by weight based on the total detergent bar composition.

This invention relates to detergent bars containing soap which do not react with the curd-forming components of hard water to form insoluble soaps. The bars may, in addition, contain a nonsoap synthetic detergent.

It is well known that the use of ordinary toilet soaps in hard water gives rise to the formation and precipitation of insoluble fatty acid salts, commonly referred to as "lime soaps." These precipitated lime soaps tend to coagulate and form a sticky curd, which is especially noticeable in washstands, bathtubs, and the like, where it rises to the surface of the water and adheres around the tube or wash basin as a ring. In laundry applications the scum or curd affects the laundry tub in like manner but, in addition, adheres to the clothes. As a result, the clothes take on a gray, dingy appearance, develop spots upon ironing, and often a rancid odor. Similarly, when used for washing the hair, lime soaps are deposited thereon, giving the hair a coarse feeling and a dull appearance.

It has now been found that lime soap formation and precipitation can be substantially avoided by incorporating in the soap, e.g., a tallow soap, a minor but effective amount of a water-soluble salt of thiodisuccinic acid



in which at least two hydrogen atoms of the carboxyl groups have been replaced by a metal selected from the group consisting of the alkali metals and magnesium.

More specific examples of lime soap dispersants are dimagnesium thiodisuccinate, disodium and dipotassium thiodisuccinates, trisodium and tripotassium thiodisuccinates, and tetrasodium and tetrapotassium thiodisuccinates.

It has further been found that a thiodisuccinic acid salt of the type contemplated is effective to inhibit or prevent curd formation without substantially impairing the foam properties of the soap. The lime soap dispersing agent of the present invention is effective in amounts ranging from about 5 to 25 percent by weight, based on soap and lime soap dispersing agent.

The soap which can be used in accordance with the present invention is not critical. Any of the water-soluble

## 2

curd-producing soaps in bar form normally used in industrial laundering, and toilet applications are contemplated. As is known, these soaps can be prepared from a variety of fatty and oily materials, such as tallow, coconut oil, cottonseed oil, corn oil, soybean oil, olive oil, palm oil, lard, greases, fish oils, and the like. The cation portion of the soap is so selected as to impart sufficient hardness to the soap to form a bar. Thus, the cation can be sodium, potassium, or nitrogen-containing, such as the ammonium soaps or those derived from triethanolamine. In general, water-soluble sodium salts of fatty acids derived from tallow and coconut oil are preferred because of the ease with which they can be formed into a bar.

As indicated earlier, the invention also encompasses ternary mixtures of soap, of the type hereinabove described, a thiodisuccinic acid salt of the type specified, and a non-soap synthetic detergent.

It has been proposed in the past to use nonsoap synthetic detergents, such as the organic alkyl sulfonates, alkyl sulfates, and alkyl benzene sulfonates, admixed with soap, to decrease its curd-forming tendency when used in hard water. Even here, however, the problem of lime soap formation and precipitation is not satisfactorily overcome.

25 The synthetic detergent component, like the soap, is also not critical. Broadly, it falls within the class of surface-active materials which are the water-soluble salts, such as the sodium or magnesium salts, of organic sulfonic acids and of aliphatic sulfuric acid esters. In other words, 30 synthetic detergents are contemplated which are water-soluble salts of organic sulfuric reaction products having in the molecular structure either a sulfonic acid or sulfuric acid ester radical.

As more specific examples of satisfactory synthetic detergents, there can be mentioned the water soluble salts, such as the sodium or magnesium salts, of alkyl benzene sulfonates, in which the alkyl groups are of branched chain structure or of linear, or straight chain, structure, having an average of 8, preferably 10, to 15 carbon atoms 40 in the alkyl radical; the water-soluble salts of alkyl sulfuric acid, having 8 to 18 carbon atoms in the alkyl group; the water-soluble salts, such as the alkali metal salts of sulfuric acid esters of primary normal aliphatic alcohols containing 10 to 18 carbon atoms, such as lauryl and oleyl alcohol; primary and secondary alkyl sulfates having pronounced detergent power and obtained from primary or secondary alcohols and olefins. Other examples of the synthetic detergent component include the sulfuric acid esters which are the water-soluble salts of sulfuric acid esters of polyhydric alcohols incompletely esterified with high molecular weight soap-forming carboxylic acids, such as the 50 water-soluble salts of sulfuric acid esters of higher molecular weight fatty acid monoglycerides, more specific examples being sodium glyceryl monolaurate sulfate and potassium glyceryl monopalmitate sulfate.

55 The method of addition of the additive of the present invention is not critical. It thus can be added to the crutcher after the soap has been made by saponification of fats. Or the additive can be added to soap chips and detergent in the amalgamator, if desired, along with other soap additives conventionally used, such as coloring agents, perfume, fillers, and the like.

The ternary mixtures of the invention will generally comprise, in weight percent, based on soap, synthetic detergent, and lime soap dispersant, 5 to 90, preferably 60 to 80, soap; 5 to 90, preferably 10 to 30, nonsoap synthetic detergent; and 5 to 25, lime soap dispersant.

In evaluating a satisfactory lime soap dispersant, a good method and the one used in the examples hereinbelow appearing is as follows: A stock solution of the test dispersant is prepared by dissolving 1 part by weight of the dispersant in 99 parts of distilled water. Stock solutions of tallow soap\* and of the various synthetic detergents are also prepared, again the concentration of the organic material in the solution being 1% by weight.

Since the stock solutions are made up to the same concentration, the relative amount of each solution deter-

Combination soap-nonsoap detergent bars containing the thiodisuccinic acid salt of the present invention were evaluated by handwashing in hard water. The tests tabulated in Table II were carried out by a panel of three persons. Judgments were made as to how much lather and how quickly it formed compared with commercially available good quality toilet soap. Also subjectively determined was the quantity of lime soap curd remaining after washing of the hands in 1 liter of 200 and 300 p.p.m. 10 hard water as compared with an unmodified bar. The various bars were rated as being "excellent," "good," "fair," and "poor" as indicated.

In making the bars of Table II, tallow and coconut soaps were grated into chips which were dry mixed with

TABLE II.—COMBARS CONTAINING THIODISUCCINIC ACID SALTS

| Ex. No. | Soap            | Conc. (Wt. Percent) | Detergent                                                                                  | Conc. (Wt. Percent) | Dispersant                  | Conc. (Wt. Percent) | Lather Quickness | Lather Quantity | Lime Soap Dispersability |
|---------|-----------------|---------------------|--------------------------------------------------------------------------------------------|---------------------|-----------------------------|---------------------|------------------|-----------------|--------------------------|
| 11      | Tallow/Coconut  | 43/29               | Sodium Alkyl Benzene Sulfonate <sup>1</sup>                                                | 14                  | Tetrasodium Thiodisuccinate | 14                  | Good             | Good            | Excellent                |
| 12      | do              | 80/20               | None                                                                                       | 20                  | None                        | Poor                | Fair             | Poor            |                          |
| 13      | do <sup>2</sup> | 59/14               | Sodium Alkyl Benzene Sulfonate <sup>1</sup>                                                | 15                  | do                          | Good                | Good             | Fair            |                          |
| 14      | do              | 42/28               | Sodium Alkyl Benzene Sulfonate <sup>1</sup>                                                | 15                  | Dimagnesium Thiodisuccinate | 15                  | do               | do              | Excellent                |
| 15      | do              | 56/14               | Sodium Alkylbenzene Sulfonate <sup>1</sup> —Magnesium Alkyl Benzene Sulfonate <sup>1</sup> | 10                  | Tetrasodium Thiodisuccinate | 10                  | Fair             | do              |                          |
| 16      | do              | 42/28               | Sodium Alkyl Benzene Sulfonate <sup>3</sup>                                                | 15                  | do                          | 15                  | do               | Good            | do                       |

<sup>1</sup> Alkyl group is polypropylene of an average molecular weight of 265.

<sup>2</sup> Contains 7% of lauric-myristic diethanolamide as a foam booster.

<sup>3</sup> Alkyl group is a mixture of straight chain alkyl groups containing 10 through 13 carbon atoms.

mines the relative percents of tallow soap or tallow soap plus synthetic detergents and dispersant for each test. For example, a 10% dispersant test is carried out as follows: Place 1 ml. of the dispersant solution and 9 ml. of the tallow soap containing solution in the bottom of a 100 ml. stoppered graduate cylinder and swirl it gently. When well mixed, dilute with 90 ml. of 334 p.p.m. hard water (2 parts calcium to 1 part magnesium, calculated as carbonates) at 110° F. The final hardness is 300 p.p.m. The graduate is then shaken vigorously for 15 seconds, and then allowed to stand for 5 minutes. At the end of this time, the milliliters of curd are measured and recorded.

The following tabulated examples illustrate the practice of the invention.

the other ingredients. After thorough mixing, the compositions were milled about 8 times, water being added where necessary to facilitate milling. The resulting homogeneous masses were stamped into bars at a pressure of 200 p.s.i.

Referring to Table II, untreated bars have inferior properties regarding lather and curd formation (Experiment 12). Combars composed of soap and nonsoap synthetic detergents give slightly better results (Experiment 13), but not so good as the combars treated in accordance with the present invention (Experiments 11 and 14-16).

What is claimed is:

1. A detergent bar having good lime soap dispersing characteristics, and suitable for use in hard water, con-

TABLE I.—LIME SOAP DISPERSANTS

| Ex. No. | Compound                                                    | Conc. | Soap         | Conc. | ml. Curd |
|---------|-------------------------------------------------------------|-------|--------------|-------|----------|
| 1       | Tetrasodiumthiodisuccinate                                  | 5     | Tallow Soap  | 100   | 10       |
| 2       | do                                                          | 4     | do           | 95    | 0        |
| 3       | do                                                          | 5     | do           | 96    | 1        |
| 4       | do                                                          | 10    | do           | 95    | 0        |
| 5       | Disodiumthiodisuccinate                                     | 5     | do           | 90    | 0        |
| 6       | Igepon T (Sodium N-Methyl-N-oleic acid taurate)             | 5     | do           | 95    | 3        |
| 7       | Dimagnesiumthiodisuccinate                                  | 10    | do           | 90    | 0        |
| 8       | Commercial Sodium Polypropyl-enebenzene Sulfonate Detergent | 20    | do           | 80    | 10       |
| 9       | Tetrasodiumthiodisuccinate                                  | 5     | Coconut Soap | 95    | 0        |
| 10      | Igepon T (Sodium N-Methyl-N-oleic acid taurate)             | 7     | Tallow Soap  | 93    | 0        |

Referring to Table I, it is noted that considerable curd formation occurs with untreated soap (Experiment 1). A combar composed of commercial sodium polypropyl-enebenzene sulfonate detergent and soap without lime soap dispersant is also unsatisfactory (Experiment 8). The lime soap dispersant of the present invention (Experiments 2, 3, 4, 5, 7 and 9) are just as effective, if not more so, than commercially available lime soap dispersant Igepon T (Experiments 6 and 10).

sisting essentially of water-soluble soap normally having poor lime soap dispersing characteristics and, as a lime soap dispersant, a water-soluble salt of thiodisuccinic acid, having at least two hydrogen atoms of the carboxyl groups replaced by a metal selected from the group consisting of the alkali metals and magnesium, said lime soap dispersant being present in an amount of about 5 to 25 percent by weight, based on lime soap dispersant and soap.

2. A detergent bar according to claim 1, wherein the lime soap dispersant is tetrapotassium thiodisuccinate.

3. A detergent bar according to claim 1, wherein the lime soap dispersant is tetrapotassium thiodisuccinate.

4. A detergent bar according to claim 1, wherein the lime soap dispersant is disodium thiodisuccinate.

\* Sodium tallow soap had 5.5% water, and on acidification and extraction with petroleum ether gave 85.6% fatty acids. The fatty acid portion had an acid number of 202 and an iodine number of 50, and contained 2% lauric acid, 4% myristic acid, 33% palmitic acid, 22% stearic acid, and 39% oleic acid.

5. A detergent bar according to claim 1, wherein the lime soap dispersant is dimagnesium thioldisuccinate.

6. A detergent bar having good lime soap dispersing characteristics, and suitable for use in hard water, consisting essentially of a water-soluble soap, a water-soluble nonsoap synthetic detergent salt of an organic sulfuric reaction product having in its molecular structure a member selected from the group consisting of sulfonic acid and sulfuric acid ester radicals, and, as a lime soap dispersant, a water-soluble salt of thioldisuccinic acid having at least two hydrogen atoms of the carboxyl groups replaced by a metal selected from the group consisting of the alkali metals and magnesium, the aforesaid ingredients being present in proportionate amounts by weight percent based on soap, lime soap dispersant, and synthetic detergent ranging from 5 to 90, soap; 5 to 90, nonsoap synthetic detergent; and 5 to 25, lime soap dispersant.

7. Detergent bar according to claim 6, wherein the synthetic detergent is alkyl benzene sodium sulfonate having 10 to 15 carbon atoms in the alkyl groups.

8. A detergent bar according to claim 7, wherein the ingredients are present in proportionate amounts of 60 to 80 percent soap, 10 to 30 percent synthetic detergent, and 5 to 25 percent lime soap dispersant.

9. A detergent bar according to claim 8, wherein the lime soap dispersant is tetrasodium thioldisuccinate.

10. A detergent bar according to claim 8, wherein the lime soap dispersant is dimagnesium thioldisuccinate.

11. A detergent bar according to claim 8, wherein the lime soap dispersant is disodium thioldisuccinate.

#### References Cited

##### UNITED STATES PATENTS

|    |           |        |          |       |         |
|----|-----------|--------|----------|-------|---------|
| 15 | 2,737,525 | 3/1956 | Mulvaney | ----- | 260—537 |
|    | 3,232,879 | 2/1966 | Lew      | ----- | 252—121 |

LEON D. ROSDOL, *Primary Examiner.*

B. BETTIS, *Assistant Examiner.*

UNITED STATES PATENT OFFICE  
CERTIFICATE OF CORRECTION

Patent No. 3,355,389

November 28, 1967

David M. Marquis

It is hereby certified that error appears in the above numbered patent requiring correction and that the said Letters Patent should read as corrected below.

Column 1, line 34, for "tube" read -- tub --; columns 3 and 4, TABLE I, second column; line 4 thereof, for "do" read -- Tetrapotassiumthiodisuccinate --.

Signed and sealed this 31st day of December 1968.

(SEAL)

Attest:

Edward M. Fletcher, Jr.

Attesting Officer

EDWARD J. BRENNER  
Commissioner of Patents